

Nov. 15, 1949

J. R. ERICKSON

2,488,276

GRINDING WHEEL

Filed Dec. 28, 1943

2 Sheets-Sheet 1



Fig. 1



Fig. 2



Fig. 3



Fig. 4



Fig. 5

JOHN R. ERICKSON

Attorney

By William T. Kiesner

Nov. 15, 1949

J. R. ERICKSON

2,488,276

GRINDING WHEEL

Filed Dec. 28, 1943

2 Sheets-Sheet 2



Inventor  
JOHN R. ERICKSON

By William T. Kneamer

Attorney

## UNITED STATES PATENT OFFICE

2,488,276

## GRINDING WHEEL

John R. Erickson, Worcester, Mass., assignor to  
 Norton Company, Worcester, Mass., a corpora-  
 tion of Massachusetts

Application December 28, 1943, Serial No. 515,907

4 Claims. (Cl. 51—296)

1

This invention relates to abrasive articles, such as grinding wheels, particularly abrasive articles utilizing diamond particles as the abrasive and to a method of producing the same.

One of the objects of this invention is to provide an abrasive article of the above-mentioned character that will be strong and efficient in action, long-lasting, and capable of facility of manufacture with facility of control of its structural characteristics. Another object is to provide a practical and dependable method for producing abrasive articles of the just-mentioned character.

Another object is to provide an abrasive article, particularly a grinding wheel, in which the abrasive portion and its supporting portion are structurally and functionally so inter-related to each other as to facilitate shaping, or facilitate change in shaping of, particularly the backing or supporting portion, by the user of the grinding wheel, to meet varying requirements of practical use, all without impairment of the structural and functional integrity of the abrasive article or grinding wheel as an entity. Another object is to provide an abrasive article, particularly a grinding wheel, of the just-mentioned character which can be efficiently and reliably produced out of materials, such as resins of the phenolic type, in a manner and by a practical and efficient method that dependably avoid difficulties, such as swelling during curing, that are met with if the structure is attempted to be made by heretofore known methods. Another object is to provide a grinding wheel comprising an abrasive annulus and a resinoid type of backing or support, in which there may be achieved such distribution of stress from the relatively small abrasive annulus to the relatively larger mass of the support or backing, during grinding action, as will make for longer life of the wheel, better efficiency of grinding, and greater strength of structure to stand up to the reactions from the stresses exerted at the grinding line.

Another object is to provide a method of constructing a grinding wheel of the above-mentioned character in which an improved and stronger junction between the abrasive annulus and the backing or support can be achieved in an economical, efficient and thoroughly practical manner. Another object is to provide a method of the just-mentioned character in which detrimental effects caused by change in volume or shape of the resinoid may be eliminated in a simple and dependable manner or may be pre-

2

vented from impairing the strength, durability or uniformity of the junction between the abrasive annulus and the resinoid backing or support. Another object is to provide a method and construction for dependably overcoming the defects of swelling, shrinking or the like in effecting the junction between the abrasive annulus and its resinoid backing or support. Another object is to provide a grinding wheel, particularly one employing diamond as the abrasive, in which the junction between the abrasive annulus and its resinoid support or backing is of such a structural and functional character that it remains substantially unimpaired when both abrasive annulus and support are turned down or trued to different shapes or conformations as, for example, is frequently required in certain grinding operations to shape not only the annulus but also its support to cope with a different or a particular grinding operation. Another object is in general to provide an improved grinding wheel and an improved method of achieving the same. Other objects will be in part obvious or in part pointed out hereinafter.

25 The invention accordingly consists in the features of construction, combinations of elements, arrangements of parts, and in the several steps and relation and order of each of the same to one or more of the others, all as will be illustratively described herein, and the scope of the application of which will be indicated in the following claims.

35 In the accompanying drawing in which is shown one of the various embodiments of the mechanical features of my invention,

Figure 1 is a central transverse sectional view, as seen along a diameter, of a grinding wheel made according to my invention, illustrating a 40 possible conformation which it may be given as a final step in the method or, in the field, to suit it to a particular grinding requirement;

Figure 2 is a central transverse sectional view as seen along the diameter of a grinding 45 wheel as it appears at the conclusion of other, and if desired, steps of my process;

Figure 3 is a diametrical transverse sectional view of a possible mold, showing it charged with certain ingredients, ready for a pressing operation;

Figure 4 shows the mold and certain parts of the wheel construction at the conclusion of the pressing operation;

50 Figure 5 shows the mold and the wheel part of

Figure 4 prepared for having the abrasive annulus molded in position;

Figure 6 is a central transverse sectional view as seen along the diameter of another form of grinding wheel as it appears at the conclusion of other, and if desired final, steps of another form of my process;

Figure 7 is a central transverse sectional view, as seen along a diameter, of a grinding wheel illustrating a shape or configuration which may be given the structure of Figure 6, by following certain other steps of my process; and

Figure 8 shows successive transverse sectional views, as seen along the diameter, of the successive structures corresponding to successive steps which may be pursued according to another form of my method.

Similar reference characters refer to similar parts throughout the several views of the drawings.

Certain features of my invention are better illustrated in connection with the construction, and the method of making it, of a so-called cup-shaped wheel which as shown in Figure 1 or Figure 2 comprises an abrasive annulus 10 carried by a backing or center that has a hole 11 by which the wheel can be mounted onto a driving shaft, the abrasive annulus 10 being of relatively small dimensions, for example,  $\frac{1}{2}$ " in thickness along a radius and  $\frac{1}{8}$ " in thickness in the direction of the axis of the wheel; this type of wheel, utilizing diamond grain as the abrasive in the grinding annulus 10 is intended primarily to perform a grinding operation by way of its side face 10a but in practice may be called upon to perform a grinding operation by way of another exposed face, such as the outer or peripheral face 10b which, illustratively, can be cylindrical. Diamond grinding wheels are usually employed in grinding very hard materials, such as cemented carbides, and are subjected to extremely severe reactions and stresses during the grinding operations. The reactions and stresses are ultimately absorbed by or dissipated in the backing or center which may be made sufficiently large and strong for that purpose but, because of the relatively very small dimensions of the abrasive annulus itself, these reactions and stresses can become exceedingly concentrated, particularly in the small area of the junction between the abrasive annulus and the backing or support. As a result failures, such as breakage of the abrasive annulus, separation thereof from the center or backing, and the like can occur and, moreover, the attempt to provide a wheel devoid of the above-mentioned shortcomings by the use of heretofore known methods of wheel manufacture has but emphasized the inadequacy of such methods for it has been found that factors such as swelling during curing of the material of the backing can make impossible the production of a grinding wheel capable of withstanding even a modest grinding load. Furthermore, all of these factors are aggravated by the requirement, to meet certain particular grinding needs, that the backing itself has to be shaped, with or without also shaping the abrasive annulus, by the grinding wheel user to meet requirements of certain subsequent grinding jobs or of some succeeding stage of grinding. To provide a practical, efficient and long-lasting grinding wheel, and a method of making it, that will overcome such disadvantages and defects as have just been noted is one of the dominant aims of this invention.

Referring first to Figure 3, I provide a mold

which may comprise an outer mold ring 12 having a bottom plate 13 and a top plate 14 provided with central holes 15 and 16 for receiving a central arbor 17, all constructed in known manner to be receivable within a suitable pressure-applying apparatus, such as an hydraulic press; thus the press may have a lower platen 18 upon which rest the bottom plate 13 with its arbor 15 and the mold ring 12, and an upper platen 19 which engages the top plate 14.

In such a mold, with the platens adequately separated and the top plate 14 removed, I place a suitable mixture of uncured resinoid with a suitable filler, and an illustrative mixture may comprise powdered uncured phenolic aldehyde resin, such as Bakelite, more specifically uncured Bakelite powder, known as BM 261. The powdered resin is preferably of fine size, for example, 220 grit size, and illustratively may be used in an amount about 86.3% by weight and thoroughly mixed with 13.7% by weight of a pigment (which may, incidentally, function also as a filler), such as manganese oxide ( $MnO_2$ ), 2.3 cc. of furfural per 100 grams of the Bakelite powder, 2.3 cc. of Carbosota per 100 grams of the Bakelite powder, and 1.6 grams of  $CaO$  per 100 grams of the Bakelite powder.

The just-mentioned proportions are illustrative and may be varied according to circumstances, and the ingredients mentioned are also illustrative. For example, I may use pyrolusite which is 90% manganese oxide and 10% impurities of various kinds.

The furfural, which is a plasticizer and hardening agent for the resin, is first mixed with the manganese oxide and that mixture is then added to, and mixed with, a mixture of  $CaO$  and the powdered uncured resin, and finally the Carbosota is added; the latter is a neutral creosote oil which aids in giving good working consistency to the resultant mix. This sequence of steps is preferred, for the manganese oxide thins out the furfural and there is avoided the difficulty and other disadvantages that would result if the furfural were added directly to the powdered resin, this latter procedure usually resulting in a sticky, lumpy mix. The resultant mix has uniformity of consistency and wetness and is sufficiently pourable for charging the molds. Also, such a mix when suitably molded and cured to form a back or center is substantially non-porous, is strong and of the right kind of rigidity, and moreover, can be turned or trued, as with an abrasive stick or other suitable tool, with comparative ease or facility, leaving a nice finish and it also takes a nice polish; it may, however, have porosity, illustratively a porosity on the order of 10%. In making up the mix, suitable screening may be resorted to, if desired, and is preferred, particularly for cold-pressing of the mix.

The above-mentioned resin BM 261 comprises essentially a mixture of phenol formaldehyde resin (about 60% by volume) which is in a partially cured state, clay or asbestos or other suitable filler (about 40% by volume), and a suitable amount of black dye; it is intended as a hot-molding material, but I am enabled to employ it for cold-molding or cold-pressing. It is less reactive than Bakelite 2417. Other suitable resins as later mentioned may, however, be employed. Such an uncured mix is placed into the mold of Figure 3, as indicated at 21, that is, in the annular space above the bottom plate 13 and between the arbor 17 and the mold ring 12 to a depth about twice the thickness of the ultimate

center or backing, the amount thus depending upon how thick it is desired to have the ultimate center or backing of the wheel. Where BM 261 resin is employed as in the above illustration, it is preferable to charge it into the mold within a short time after making up the mix, for example, within one or two hours, to avoid the effects of drying out and other possible undesirable actions. With a suitable template the top surface is levelled off throughout the major portion of its radial extent from the center outwardly, as indicated at 22, the template being shaped, however, to give the outer top portion of the uncured resinoid charge 21 a frusto-conical surface as indicated at 23.

This operation is carried on, of course, with the top plate 14 removed and any suitable means (not shown) may be used to aid the operator in swinging and guiding the template about the axis of the arbor 17 so that it will leave the top surface 22 and the frusto-conical surface 23 of the resinoid charge 21 free from material irregularities or undulations, make them both concentric with each other and with the mold, the top face 22 thereby falling in a plane that is transverse to the axis of the mold. The mix, though wet and pourable as above described, is however not of such fluidity as will cause such flow of the upper portions of the charge 21 as would materially alter the shape given the charge by the above-mentioned template; in other words, the consistency of the mix 21 is sufficiently thick, though plastic, for the charge to maintain its shape at least until the annular tri-angularly-cross-sectioned space S between the surface 23 and the mold ring 12 is filled up.

Into the space S I now place an uncured mix which, from the viewpoint of curing and union therewith, is compatible with the uncured ingredient or ingredients of the charge 21 in the mold and where, as in the above-described illustration the charge 21 is also an uncured phenolic resinoid mix, I make up a resinoid mix with which to charge the space S that comprises also an uncured phenolic resin, but this mix I make up to have, when cured, a suitable porosity, for reasons later explained in greater detail. This second mix is, however, also related as to various of its attributes to the later-described mix out of which I make up the abrasive annulus 10.

The mix to fill into the space S of Figure 3 illustratively comprises 30.48% by weight of powdered uncured phenolic resin or Bakelite, more specifically, Bakelite resin known as "BR 9727," a suitable filler, preferably a mineral filler in particle form such as feldspar of, for example, 220 grit size, or ground quartz, or the like, and where feldspar is used its amount is 63.80% by weight, 3.60% by weight of CaO, 2.12% of carbon black (to function as a pigment, the manganese oxide used in the charge 21 being a black pigment), furfural in the proportion of 50 cc. per pound of uncured powdered resin, and Carbosota in the proportion of 30 cc. per pound of the above-mentioned uncured powdered resin. This mix is poured into the space S which by way of illustration in Figure 3, assuming that the outside diameter of the charge 21 is 6", is in cross-section a right-angled triangle whose vertical leg and horizontal leg are each about  $\frac{1}{2}$ " in length. Actually, in one embodiment of my invention for a 6" wheel, the charge 21 consisted of 625 grams and the charge indicated in Figure 3 at 24 of the just-described mix for the annular space S consisted of 30 grams. The charge 24 is, of course, levelled

off at the top, as with a template, to bring its top face 25 into the same plane with the top face 22 of the charge 21.

The operations thus far described may be and preferably are carried on with the mold parts and platens cold, that is, at about room temperature, the top plate 14 is put in position about the upper end of the arbor 17 and within the upper end of the mold ring 12, whence the pressure-applying apparatus is actuated, as by moving the platens 18 and 19 one toward the other to telescope the top plate 14 toward the bottom plate 13 to reduce the axial dimension of the charge 21 to about one-half, and this may require a pressure on the order of 5 tons per square inch. This pressing operation may be and preferably is carried on with the mold parts and platens cold.

At the conclusion of this pressing operation the parts are in the relative positions shown in Figure 4 from which the change in shape of the charges 21 and 24 can also be seen, the charge 21 of Figure 3 being now compressed axially to the proportions shown at 21a in Figure 4 while the charge 24 in the space S of Figure 3 is compressed axially into the shape shown at 24a, but will be seen not to be materially altered insofar as the shape and area of its upper face 25 are concerned, the pressing operation, of course, neatly merging that upper face 25 into the upper face 22 of the compressed charge 21a, a similar nicely of merging taking place between the outer cylindrical faces of the two charges 21a and 24a in Figure 4. Also the two compatible uncured mixes are, under this relatively high pressing together, brought into intimate inter-mingling in the region, indicated by the inclined line or plane 26 in Figure 4, of their mutual contact, all in a manner that is conducive, during the curing or heat treatment, for the two portions 21a and 24a to cure and harden into a single entity devoid of any material line or plane of cleavage therebetween.

The top plate 14 is now removed whence it is replaced by a top plate 14a as shown in Figure 5 top plate 14a being of lesser radius than the radius of the mold ring 12 by an amount equal to the radial dimension which the abrasive annulus 18 (Figures 1 and 2) is to have, and in the illustrative embodiment here selected for description, that dimension is to be  $\frac{1}{8}$  of an inch. Accordingly, I may now charge the annular space 27 (Figure 5) above the portion 24a and between the mold ring 12 and the top plate 14a with an abrasive and bond mix, indicated in Figure 5 at 28. Here it is to be noted that I prefer, in shaping the space S during the steps described above in connection with Figure 3, to make the radial dimension of the upper face 25 of the charge 24 several times greater than the radial dimension which the abrasive annulus 18 is to have; in the illustration the former is  $\frac{1}{2}$ " and the latter is  $\frac{1}{8}$ ".

The mix represented by the charge 28 in Figure 5 is in turn compatible, as to curing and certain other characteristics, with the mix of which the charge 24 of Figure 3 is made. In place of the illustrative 63.80% of feldspar, I employ, where the abrasive annulus is to contain diamond as the abrasive, 41.00% by weight of diamond particles and 25.50% by weight of quartz particles, then 25.47% by weight of powdered uncured Bakelite, namely, BR9727, 2.97% by weight of CaO, 3.26% by weight of furfural, and 1.80% of Carbosota, the furfural and Carbosota, though being set

forth in percentages by weight, are nevertheless in amounts equivalent to 50 cc. of furfural per pound of the powdered resin and 30 cc. of Carbosota per pound of the powdered resin.

This abrasive and bond mixture I pour into the annular space 27 of Figure 5 and level off as by a template to a height about twice the axial dimension which the abrasive annulus 10 of Figures 1 and 2 is to have in the final product and where the latter dimension is to be  $\frac{1}{8}$ ", the charge 28 in Figure 5 may have a height or depth of about  $\frac{1}{4}$ ".

Bearing in mind that the portion 24<sup>a</sup> in Figure 5 is still uncured, I now place into the annular space 27 and above the charge 28 a mold ring 29 and bring the pressing apparatus into action, as by suitably actuating the platens 18 and 19 as before, thus pressing the charge 28 downwardly in the annular space 27 of the mold and against the upper face 25 of the compressed but uncured portion 24<sup>a</sup>.

Here a pressure on the order of 5 tons per square inch may be employed, bringing the axial dimension of the charge 28 down to about  $\frac{1}{2}$ , illustratively to about  $\frac{1}{8}$  of an inch; at the same time the mutually engaging parts of the portions 28 and 24<sup>a</sup> are forced, under this substantial pressure, into an intimacy of inter-mingling and inter-engagement throughout the area 30 of their respective potentially-reactive and compatible resinous constituents as is effective, during the subsequent curing, to cause these parts to join and harden and cure together as though they were a single entity, somewhat the same as takes place when the charges 24 and 21 of Figure 3 are compressed as was above described.

Having completed this last-described pressing operation, the uncured wheel structure is stripped from the mold and is then heat-treated to cure the resinoid and harden the three portions of the wheel into a single unitary strong entity. As stripped from the mold the structure has dimensions or shapes substantially like that shown in Figure 2. Heat treatment may take place in an oven and is suited to the particular characteristics of the resin employed in the mixes and with the resins and mixes illustratively set forth above, a suitable heat treatment comprises heat treatment of the structure at about 100° C. for a period of about 5 hours followed by treatment at about 175° C. for about 24 hours.

The resultant wheel structure appears as shown in Figure 2. It is characterized by substantial strength throughout, by freedom from detrimental or material warping, shrinkage or swelling, and by uniformity of strength particularly in the rather concentrated region where the three portions 21<sup>a</sup>, 24<sup>a</sup> and 10 (Figure 2) are merged into a single solid entity. It has heretofore been impracticable or difficult to achieve satisfactory union between such a small or concentrated abrasive annulus as the annulus 10 and a backing or support, and this has been due principally to the fact that change in volume, as by swelling, during curing, causes such distortion or relative shift as to preclude uniformity of strength of the union between the abrasive annulus and its support; accordingly, the abrasive ring or annulus would fail because of failure at a weak spot or region in the annular area throughout which the two parts are supposed to be in union. This defect became aggravated when the wheel structure, particularly the resinoid backing or center, was turned down or trued to a different shape such as, for example, the general type

of configuration shown in Figure 1, and here it is to be noted that such change in shape was frequently effected by the user. Such limitations and deficiencies of prior practices and constructions have also imposed a limitation upon the hardness that could be given the abrasive annulus itself or the backing or center or both, because, in the effort to overcome such deficiencies lesser pressures have been employed in the pressing operations, and curing temperatures and periods have been employed which, while tending to mitigate such deficiencies, precluded the achievement of a hardness that is desirable from structural and operating viewpoints.

Such and other deficiencies, limitations and disadvantages my invention overcomes, and for various reasons. For example, the portion 24<sup>a</sup> in Figure 2, compounded and proportioned in relation to the other parts of the wheel as illustratively above set forth has a porosity which, during curing, coacts to prevent distortion, as by swelling, of the abrasive annulus portion in that gases or vapors that might be evolved as the abrasive mix cures, instead of blistering or raising the abrasive mix away from the portion 24<sup>a</sup>, find egress across the plane of contact between the two and into and through the pores of the part 24<sup>a</sup>. As a result, the abrasive mix and the portion 24<sup>a</sup> can undergo curing virtually as a single homogeneous mix would undergo curing and hence the union between the two is strong and uniform throughout. A similar action can take place in effecting a like, strong and uniform union between the portions 21<sup>a</sup> and 24<sup>a</sup>, but due to the preferred configurations or relative contact areas employed in assembling the several mixes, the union between the portion 24<sup>a</sup> and the portion 21<sup>a</sup> is over an area of inter-mingling or engagement between the two mixes that is greatly in excess of the area throughout which the abrasive mix and the portion 24<sup>a</sup> are inter-mingled at their region of contact; in the illustrative embodiment, the former area is about four times as great as the latter area, and desirably an angularity, like that indicated in Figure 2, is provided between the two.

Furthermore, because of this divergence in areas the mix employed in making up the backing or center 21<sup>a</sup> may differ considerably from the mix employed in making up the part 24<sup>a</sup>, though preferably maintaining compatibility of the uncured resins employed so as to facilitate what is practically a curing of the two as a single mix. Thereby the mix for the center or back 21<sup>a</sup> may be compounded, illustratively as above set forth, and cured, to give it the desired hardness, rigidity, strength and other mechanical properties desired, for the larger area of inner engagement, as at 26 in Figure 4, can still form in the aggregate an adequately strong union while the porosity in the portion 24<sup>a</sup> provides egress for such gases or vapors as are evolved in the mix 21<sup>a</sup> undergoing curing, thus preventing change in volume with accompanying distortion or other phenomena as might disrupt the uniformity of the union between the two. An illustrative porosity for the portion 24<sup>a</sup> is 15 percent; another is 4 percent.

Preferably also, and as the above illustrative compositions of the mixes for the parts 10 and 24<sup>a</sup> indicate, the two mixes have substantially identical or closely similar compositions structurally; that is to say, in each are present substantially the same proportions of resin, furfural, Carbosota, CaO and of feldspar (with carbon black) filler on the one hand and diamond grain plus quartz grain on the other hand. As a result

there is excellent compatibility between the two as to curing characteristics and phenomena that transpire during curing, and in the resultant integral cured final structure, the two portions 10 and 24<sup>a</sup> have substantially the same structural characteristics mechanically, resulting in similarity of action and reaction under the stresses and strains of practical use. Thereby, also, the portion 24<sup>a</sup> in Figure 2 is of a structural character to dependably and reliably transmit and distribute to the center or backing 21<sup>a</sup> such strains and stresses, in effect substantially relieving, and certainly lessening, a too direct concentration of strains or stresses in the region of the area 30 throughout which the uncured mixes 28 and 24<sup>a</sup> of Figure 5 became engaged and intermingled. These substantial similarities of the above-mentioned characteristics of the mixes 28 and 24<sup>a</sup> in Figure 5 also coact toward giving these two mixes, during curing, similar or substantially identical change of volume characteristics whereby also curing of the two into an integral or single entity, without material risk of cleavage, shear, rupture or the like along the annular area 30 is avoided or lessened. Preferably the compounding of the several mixes includes, as in the illustrations given above, an ingredient such as CaO which coacts with water or water vapor evolved during the curing to chemically take it up and thus counteract material change in volume by shrinkage.

The wheel may be used in the form shown in Figure 2 but more usually, before shipment, the wheel is mounted in a suitable apparatus and rotated and the hardened cured back or center 21<sup>a</sup> turned down to change its shape, as by use of an abrasive stick, though the user of the wheel may himself in a similar way change the shape of the wheel. In Figure 1 I have indicated at 21<sup>b</sup> and at 24<sup>b</sup> an illustrative change in conformation which may be given the parts 21<sup>a</sup> and 24<sup>a</sup> of Figure 2, the turning down or truing being in a direction to emphasize the dish or cup shape of the wheel as might be necessary to suit it to some particular grinding operation. The cured portion 24<sup>b</sup> lends itself readily to such a turning down operation and the shape initially given it as in Figure 2 will be seen to be such as to make it possible to maintain the now diminished annular area 26<sup>a</sup> in Figure 1 as compared to the area 26 in Figure 2 (still greater than the annular area 30). In the shape shown in Figure 1 the abrasive annulus 10 may be made to operate by way of any of its three exposed faces and by suitable truing tools, such as an abrasive stick, these or any of them may be changed in shape or conformation to suit particular grinding needs.

The ease of change in conformation or shape makes it possible also for the user to vary the conformation to suit particular grinding needs, and though the abrasive annulus itself may be thus reduced to small radial dimension, the underlying portion 24<sup>b</sup> strengthens and reinforces it and gives it good and substantial support to and from the backing 21<sup>b</sup> itself.

In making up the mix for the charge 24 in Figure 3, I may employ other fillers and preferably I employ fillers that are relatively low on the scale of hardness; thus a preferred filler is cryolite which has a hardness on the order of 2.5, or pyrolusite which has a hardness on the order of 2.0, or powdered metal of which aluminum is a good illustration, the latter having a hardness on the order of 2 or 3, and also I may employ certain clays. The fillers to employ are hence preferably soft, and preferably they do not re-

act with the bond and preferably also they are not hygroscopic. By following these preferred characteristics for the filler, the final cured portion of the wheel, such as the part 24<sup>a</sup> of Figures 2 and 4, after curing, can be easily and readily turned down to give it any desired shape, by the use, for example, of an ordinary so-called "abrasive stick," and, for certain purposes, the hardness of the filler employed should be below that value which would cause that portion of the wheel to take the edge off of certain tools, such as a tool made of Carboloy.

Also it is preferred that certain relationships as to porosity be maintained as earlier above set forth and it is preferred also that the volume percentage of the bond in the mixes 24 and 28 be substantially the same, these factors coacting to achieve good adhesion or a good union between the portions 10 and 24<sup>a</sup>, as seen in Figure 2. The mix 21 may and preferably is given a suitable porosity, say, on the order of 10%, and the provision of suitable porosities in the several sections or portions aids in combatting swelling or tendencies toward swelling, for the porosity can provide sufficient egress for or accommodation of such gases or vapors as are evolved during curing, and thus detrimental or undesired changes in volume, particularly such as might have bad effects upon the union between adjacent portions, can be prevented or minimized.

With such relationships also, a greater range of variation or flexibility in the structural relationships and also in the method of making up the wheel are achieved. For example, it is possible to first cure the structure as it appears in Figure 4, in any suitable way, and after curing, mold thereon the abrasive mix or annulus 10, following steps substantially like those described above in connection with Figure 5, and then subjecting the now composite and complete structure, of which the parts 21<sup>a</sup> and 24<sup>a</sup> are already cured or, if preferred, substantially cured, to suitable heat treatment to cure the bond of the abrasive annulus. By way of illustration, the two steps of curing can be and preferably are, as to heat treatment, the same and each curing step may comprise heat treatment at about 100° C. for a period of about 5 hours followed by treatment at about 175° C. for about 24 hours. The heat treatments preferably take place in an oven, the composite wheel center or back being restored to the mold apparatus after curing in order to have the mix of the abrasive annulus molded and pressed thereon.

The security of union or of junction between the several parts achievable according to certain features of my invention and also the ease and facility with which shaping after curing, particularly of the part that corresponds to the mix 24, makes possible the carrying out of certain features of my invention in other forms. For example, instead of shaping or molding, pressing, and curing the wheel structure with its several portions shaped as shown in Figure 2 and as above described, the wheel structure may be made up as indicated in Figure 6 in which the backing, indicated at 30, is a substantially plain disk and has the abrasive annulus 10 mounted thereon by the interposed portion 31, the three portions being compounded as to their respective mixes in the manner above described. By the use of appropriate molds or mold parts or rings, the three mixes may be molded and pressed together "green," and then cured, as by removal from the mold and baking. Or portions 30 and 31 may be

molded and pressed together "green," cured, and then the abrasive element 10 molded and pressed thereon and the resultant unit cured, as by baking; the latter method has advantages in that, after curing the entity 30-31, the ease with which the parts may be turned down or trued, as by an abrasive stick, makes it possible to give that part or face of the portion 31 any desired configuration, shape or dimension as, for example, might be appropriate or suitable for the attachment 10 thereto or union therewith of the abrasive annulus 10.

The structure shown in Figure 6 may, like the structure shown in Figure 2, be shaped as by turning down its various surfaces or faces to the desired configuration as, for example, by truing or turning down along the broken lines 32-33 of Figure 6, giving an ultimate shape like that shown in Figure 7, or it may be conformed by turning down to the shape of the wheel shown in Figure 1 and earlier above described. The turning down along the broken line 33, in Figure 6, and particularly along that part of it that intersects the portion 31 may, if desired, be effected after the completion of curing of the entity 30-31 and hence prior to the molding and curing thereon of the abrasive annulus 10, where it is preferred to make the wheel in two steps of curing, and in such case the surface 34 of the portion 31 and to which the abrasive annulus 10 is to be joined may be shaped or turned to its desired configuration and also the outer cylindrical face of the portion 31, prior to the assemblage and curing thereon of the abrasive annulus 10.

Such features as these also make it possible to give, by truing or turning down, geometric accuracy to that face of the backing or support structure to which the abrasive annulus is to be joined and thus a number of practical advantages may be achieved. For example, departures from geometric accuracy such as may be caused by uncontrollable or accidental swelling, shrinkage, warping, or other changes, particularly during curing when the structure is cured outside of the mold, may thus be quickly and inexpensively rectified. Also, in such case particularly, wastage or inefficient use of expensive diamond abrasive can be avoided for the innermost boundary of the abrasive annulus 10 may thus be accurately determined with the result that uniformity of abrasive action by the abrasive annulus 10 continues down to and including the very last or innermost layer of diamonds thereof. These latter advantages are peculiarly practicable where the abrasive annulus is made up in the shape of a ring carried by the outer periphery of a disk-like or cylindrical center or backing and makes possible also construction of wheels of that type with simpler and less expensive molding equipment; this can be illustrated by the successive steps indicated in Figure 8.

Thus, let it be assumed that such a peripheral grinding wheel is to be made up to have an outside diameter D. In such case, by the use of any suitable molding apparatus, and hence in any known manner, I mold up two mixes, like the mixes 21 and 24 above described, to form a disk-like or cylindrical center or backing 36 with a peripherally-extending annulus 37, the union and junction therebetween being just as secure and having other attributes as were described in connection with the junction between the parts 21<sup>a</sup> and 24<sup>a</sup> of Figure 2; in Figure 8, the outside diameter of the outermost portion 37 is the dimension D, as indicated, and its radial dimension or

thickness is materially greater than the radial dimension or thickness of the ultimate abrasive annulus which the wheel is to have. For example, if the latter is to be  $\frac{1}{8}$ ", the thickness of the portion 37 can be  $\frac{1}{4}$ ".

After curing, which is preferably achieved by baking as in an oven and hence outside of the mold, the structure 36-37 is mounted on an arbor for rotation, or supported in any suitable way to be rotated about its axis, and is turned down to remove a substantial portion of the annulus 37, preferably in an amount to correspond to the radial dimension of the ultimate abrasive annulus which the wheel is to have, and the side faces of the structure may likewise be turned down and trued. The annulus 37 thus becomes in cross-section an annulus 38 with its outer face 39 turned to substantial geometric accuracy, in the illustration, a true cylinder of revolution; due to the features above described, this truing operation is an easy one to carry out, the compositions of the parts permitting ease of cutting by the truing or turning tool.

The resultant structure is now returned to the same mold which has an inside diameter of D, thus leaving an annular space between the geometrically accurate internal cylindrical face of (diameter D) of the mold ring and the geometrically accurate face 39, and into this space an abrasive mix, like that out of which the abrasive annulus 10 above described is made, is injected in suitable quantity and under suitable pressure, as by the use of a mold structure substantially like that shown in Figure 5 and utilizing a mold ring 29 to act upon the abrasive mix which thus becomes neatly and accurately conformed to the concentric cylindrical faces of the mold and the part 38. Heat treatment then ensues, preferably outside of the mold as in an oven, thus to cure the abrasive annulus which in Figure 8 is indicated at 40. After curing, either or both of the side faces of the composite backing 36-38 may be shaped as by turning or truing and, by way of illustration, turning down 45 may take place along the broken lines 41 and 42 where the abrasive wheel is to have side clearance.

The plane of the junction or union between the portions 36 and 37 can be oblique or inclined, as by making it frusto-conical as indicated at 43, thus to give the junction between the portions 36 and 38 in the final wheel a greater area than the junction between the abrasive annulus and the portion 38.

As above set forth, reference to specific resins is to be interpreted as illustrative and other resins may be employed such as, for example, other forms or compoundings of phenol formaldehyde resins, also aniline formaldehyde, any one of the alkyd resins, shellac, rubber, methyl methacrylate, glyptal, styrene, and the like, or other suitable or equivalent resins, all of which I comprehend within the term "resinoid" or "resin" or "resin-bonded" used in the claims.

It will thus be seen that there has been provided in this invention, an article, a composition and a method in which the various objects hereinabove set forth together with many thoroughly practical advantages are successfully achieved.

As various possible embodiments might be made of the mechanical features of the above invention and as the art herein described might be varied in various parts, all without departing from the scope of the invention, it is to be understood that all matter hereinabove set forth is

to be interpreted as illustrative and not in a limiting sense.

I claim:

1. A grinding wheel comprising a resinoid back presenting a ring-shaped securing face and a resin-bonded abrasive annulus spaced a short distance from the aforesaid securing face and having a ring-shaped securing face that is of lesser width than the width of the securing face of said resinoid back and a resinoid stress-distributing annulus interposed in the space between said first-mentioned securing face and said abrasive annulus and presenting annular faces respectively matching in width the different widths of said two securing faces and being joined thereto and integrally united therewith and having a cross-section that varies substantially progressively from the lesser width of said one of its securing faces to the greater width of the other securing face thereby to transmit the substantial grinding stresses exerted upon the abrasive annulus to said back and distribute them throughout the larger area of the securing face between the resinoid back and said resinoid annulus, and said resinoid annulus being cured to a porosity between about 4% and 15%.

2. A grinding wheel comprising a back made of a resinoid mix containing a filler that is relatively low in hardness and having a ring-shaped securing face, an abrasive annulus having a ring-shaped face of less width than said securing face of said back, and an interposed securing and reinforcing annulus made of a resinoid mix containing a filler that is relatively low in hardness and compounded to have a porosity for the escape of gases therethrough, said interposed annulus having faces respectively integrally united to said securing face of said resinoid back and said ring-shaped face of said abrasive annulus under conditions of heat and freed from deleterious blistering or disunion through the escape of evolved gases or vapors through the aforesaid porosity and being of substantially corresponding variation in cross-sectional configuration from one of said faces to the other, and said resinoid annulus being cured to a porosity between about 4% and 15%.

3. A grinding wheel comprising a resinoid back having a substantially frusto-conical securing and thrust-receiving face and an abrasive annulus spaced a short distance from the aforesaid face and having a ring-shaped face of less width than the width of said frusto-conical face and an annular resinoid member interposed in the space between said thrust-receiving face and said ring-shaped face for distributing, in lesser intensity throughout said thrust-receiving face, stresses from said abrasive annulus to said resinoid back and, for that purpose, having a frusto-conical face substantially matching in width said first-mentioned frusto-conical face and integrally

united thereto and having a face of lesser width to which said abrasive annulus is united throughout the ring-shaped securing face thereof, and said resinoid annulus being cured to a porosity between about 4% and 15%.

4. A grinding wheel comprising a disk-like truable resinoid back comprising a cured porous resinoid mix containing a soft filler and having a porosity on the order of 10%, said back presenting 10 a peripheral substantially cylindrical face and carrying a truable abrasive annulus having a peripheral substantially cylindrical face substantially aligned with said first-mentioned cylindrical face, said abrasive annulus being mounted upon and secured to a side face of said back by means of a truable annular layer of resinoid containing a soft filler and cured to a porosity on the order of from about 4% to about 15% and having a peripheral substantially cylindrical face substantially aligned with said first-mentioned face, 15 said layer being of greater radial dimension than that of said abrasive annulus and tapering off in thickness in a direction away from its said face to merge its exposed side face substantially with said side face of said back, thereby to distribute stresses from said annulus to and throughout a greater annular area of said back than the annular area of said annulus and whereby the last-mentioned relationship may be maintained even 20 after truing the aligned cylindrical faces or the merged side faces of said layer and of said back to a shape, such as frusto-conical, to provide clearance for said abrasive annulus, said annular layer and said back being integrally joined together throughout said greater annular area freed from deleterious blistering or disunion through the escape of evolved gases or vapors, during curing, through the aforesaid porosity of said annular layer.

JOHN R. ERICKSON.

#### REFERENCES CITED

The following references are of record in the 45 file of this patent:

#### UNITED STATES PATENTS

| Number    | Name          | Date          |
|-----------|---------------|---------------|
| 1,785,437 | Doermann      | Dec. 16, 1930 |
| 1,826,300 | Chapell       | Oct. 6, 1931  |
| 1,832,515 | Webster       | Nov. 17, 1931 |
| 2,070,734 | Voegeli-Jaggi | Feb. 16, 1937 |
| 2,073,590 | Sanford       | Mar. 9, 1937  |
| 2,110,143 | Ball et al.   | Mar. 8, 1938  |
| 2,150,886 | Van der Pyl   | Mar. 14, 1939 |
| 2,268,663 | Kuzmick       | Jan. 6, 1942  |

#### FOREIGN PATENTS

| Number  | Country     | Date           |
|---------|-------------|----------------|
| 166,869 | Switzerland | Apr. 16, 1934  |
| 178,296 | Switzerland | Sept. 16, 1935 |